

## UNITED STATES PATENT OFFICE

2,406,072

ELECTRODEPOSITION OF METALS AND  
BATH COMPOSITION THEREFOR

Kenneth M. Gaver, Columbus, Ohio, assignor, by  
means assignments, to The Ohio State Uni-  
versity Research Foundation, Columbus, Ohio,  
a corporation of Ohio

No Drawing. Application February 15, 1941,  
Serial No. 379,127

22 Claims. (Cl. 204—49)

1

This invention relates to electro-deposition of metals, and more particularly to electroplating baths containing a salt of the metal to be deposited and an addition agent for producing a bright adherent plate on the base metal.

It is an object of this invention to provide an improved electroplating bath for producing bright, smooth, uniform metal coatings in electroplating processes.

Another object is to provide an improved electroplating bath composition which comprises a colloidal solution of an amylose compound which is incorporated in sufficient amount to inhibit the building up of large crystals of metal during the electrodeposition so as to form a metal deposit having an adherent coating of high luster. These and other objects and advantages will be apparent from the following description.

My invention is particularly adapted to nickel plating, but, in its broadest aspects, is applicable as an improved plating bath for producing a smooth, uniform plate in electrodepositing other metals, such as chromium, copper, zinc, cadmium, cobalt and iron. In this connection, it has been proposed heretofore to use colloidal solutions as addition agents in nickel plating baths as brighteners but they have not been employed to a great extent because of the difficulty of controlling their effect and, in general, are restricted to use in low current density operations. A wide variety of organic and inorganic compounds has been suggested heretofore as addition agents in electroplating baths but none of these materials has been entirely successful.

According to the present invention, there is employed a metallic starchate compound which incorporates both the metal ion and starch molecule. The particular starchate compound may be selected to correspond to the metal salt which is in solution in the bath for supplying the metal to be deposited. The amount of the addition agent added may vary widely depending upon the composition of the electroplating bath, and the control or addition agent may be incorporated in the form of a powder, or preferably an aqueous solution.

My improved addition agent is produced by reacting starch with alcohol soluble hydroxides, such as sodium, potassium, and the like, under conditions such that the metallic starch alcoholate is produced wherein the alkali metal is attached through an oxygen atom to a carbon atom in the complex  $\alpha$ -glucopyranose or  $\alpha$ -gly-

2

copyranose residue. This alkali metal starch alcoholate compound, which is referred to as a metallic starchate, when dissolved in water forms a limpid solution and may be incorporated as such in an electroplating bath.

The method of making the alkali metal starchate which is used in compounding my improved electroplating baths may consist of reacting 417 pounds of flake caustic soda or caustic potash in approximately 500 gallons of industrial ethyl alcohol. The mixture is allowed to stand to precipitate the carbonate impurities present which are removed by filtration.

15 Approximately 500 pounds of dry starch (i. e. potato starch) is introduced into the alcoholic NaOH solution and the whole mixture refluxed for two hours below 98 degrees C. while being vigorously stirred. The product is then 20 filtered and washed free of alkali with ethyl alcohol and the filter product consisting of sodium starchate is dried in a vacuum oven under 78 degrees C. equipped with means for preventing entry of carbon dioxide and means for recovery of the alcohol. The dry product is 25 then ground, screened and packed in substantially airtight containers.

The sodium starchate compound formed as 30 described is readily soluble in water with spontaneous hydrolysis, whereas the original starch is insoluble.

In producing the sodium starchate, other sources of starch may be employed such as that derived from corn, wheat, potatoes, sago, arrowroot, cassava, etc.

35 Further details regarding the manufacture of alkali metal starchates and derivatives thereof, their nature, and characteristics, are given in my copending application Serial No. 357,995, filed September 23, 1940.

40 Where it is desired to employ nickel starchate, this can be formed by reacting sodium starchate with nickel chloride in alcohol forming nickel chloro starchate. This compound may be used, 45 or its amino derivative. The latter is made by reacting the nickel chloro starchate compound with ammonium hydroxide, filtering, and air drying the product to produce amino hydroxy starchate. If the amino hydroxy starchate is dried at a higher temperature nickel hydroxy starchate is produced. This merely illustrates a 50 typical example and where it is desired to use other metallic starchates than the alkali metals, 55 they may be readily made by reacting the alkali

metal starchates, such as sodium starchate, with the proper metal salt compound.

The following typical examples will further illustrate my invention, but it is understood that my invention is not limited to these particular baths, but is applicable to the preparation of various other metal plating baths depending upon the metal to be deposited.

*Example I*

|                  | Parts by weight |
|------------------|-----------------|
| Nickel sulfate   | 135-165         |
| Nickel chloride  | 20-30           |
| Boric acid       | 20-40           |
| Sodium starchate | 5-25            |

The above ingredients are dissolved in sufficient water to provide an electrolytic bath and the pH adjusted to the desired value by adding small amounts of sulphuric acid or alkali as required.

*Example II*

|                  | Parts by weight |
|------------------|-----------------|
| Nickel sulfate   | 135-165         |
| Nickel chloride  | 20-30           |
| Boric acid       | 20-40           |
| Nickel starchate | 5-25            |

The above ingredients are dissolved in sufficient water to provide an electrolytic bath as in Example I.

*Example III*

|                        | Parts by weight |
|------------------------|-----------------|
| Sodium cyanide         | 100-125         |
| Cadmium hydroxide      | 35-50           |
| Sodium sulfate         | 40-55           |
| Sodium starchate (dry) | 10-25           |

The above ingredients are readily soluble in water to form an electroplating bath. In place of the sodium starchate, cadmium starchate may be substituted similarly as in Example II.

*Example IV*

|                                         | Parts by weight |
|-----------------------------------------|-----------------|
| Copper cyanide                          | 100-120         |
| Sodium cyanide                          | 150-160         |
| Sodium carbonate                        | 25-30           |
| Sodium starchate (50% aqueous solution) | 5-20            |

The above ingredients are mixed together and may be dissolved in approximately 100 gallons of water or in an amount to produce the desired pH value solution. Copper starchate may also be used in place of sodium starchate where desired.

The amount of metallic starchate agent added in practice may vary depending upon the acidity or alkalinity of the plating bath. Nickel and other similar metal plating solutions are readily affected by the addition of the starch colloidal solution and the amounts used, as well as other details of operation, it will be understood, are regulated to produce tough, adherent, smooth coatings of the desired thickness.

In the foregoing examples, it will be appreciated that other metal salts and mixtures of different compounds may be used in formulating the plating bath and the metallic starchate used alone or in conjunction with other modifying substances, such as sulphonated oils and the like.

The metallic starchate addition agent combines the colloidal action of the starch molecule with the more reactive metal ion so as to perform the dual function of supplying an active metal ion and the colloidal dispersion properties of the starch molecule. In this manner, there is pro-

vided a novel addition agent for electroplating baths which may be used to introduce both the metal ion which is deposited from a solution and the amylaceous colloid for controlling the metal deposit to produce small uniform crystals whereby the surface of the deposit has a bright smooth appearance.

As examples of starchate compounds which may be employed as addition agents in the electroplating baths are the following:

|                     |                      |
|---------------------|----------------------|
| Sodium starchate    | Zinc starchate       |
| Potassium starchate | Tin starchate        |
| Nickel starchate    | Cadmium starchate    |
| Copper starchate    | Cobalt starchate     |
| Chromium starchate  | Iron starchate       |
| Silver starchate    | Molybdenum starchate |

The metal starchates listed are merely illustrative of the most common metal compounds which may be used. Any soluble starchate compound may be employed. Further, when desired the chloro, nitro or hydroxy starchate compound of the appropriate metal can be utilized.

The starchate compounds mentioned may be formed from the sodium starchate compound by reacting the same with the appropriate acid metal compound so as to produce a substitution product of the desired metal starchate. In this connection, many salts are soluble in ether and the reactions for making the appropriate metal starchate may be carried out in a manner similar to that indicated by the use of alcohol as a solvent. Other solvents which will dissolve the reaction ingredients may be used. In some cases, the reactions for forming the metal starchate product can be performed using water as a solvent, but where the product is to be used as a powder, the drying of the finished product becomes an important factor. Adjustment of the addition agent, or agents, of course, will be made in the acid and alkali electroplating baths in order to produce the improved results.

Further, my metallic starchate compound may be conveniently supplied and stored as a dry powder wherein the consumer may dissolve the dry powder ingredient in water and add it to the electroplating bath. Also, if desired, my addition agent may be incorporated in one or more of the ingredients forming the electroplating bath and during use, the remaining constituents of the bath incorporated and made up into a solution having the required pH value.

Alloys of various metals may also be electro-deposited from suitable combinations of salts with my addition agent made up in the proportion to produce a bright metal deposit. Alloys of nickel and iron or copper, as well as brass, may be accomplished by using a mixture of the metal salts as is conventional in the art. With the use of large amounts of my starchate compound the viscosity of the electrolyte may be increased somewhat over water and high current densities employed so that heavier deposits of metal may be formed.

It will be understood that my invention is adapted for widely different embodiments and that it comprehends various plating baths which include metal starchate compounds as brightening agents and is not limited to the particular examples given, which are merely exemplary. It is also understood that the new addition agents may be incorporated in various amounts in the different baths as required to produce the improved results.

Further, such modifications in the use of my

new brightening agents as necessitated under different conditions and uses are contemplated to be within the scope of this invention.

Having thus fully described my invention, what I claim as new and desire to secure by Letters Patent is:

1. A plating bath for the electrodeposition of metal comprising an aqueous solution providing ions of the metal to be deposited and a metal starchate addition agent comprising the reaction product of starch and an alkali metal.

2. A plating bath for the electrodeposition of metal comprising an aqueous solution providing ions of the metal to be deposited and having a colloidal solution of a starchate compound comprising the reaction product of starch and an alkali metal incorporated in said bath.

3. A plating bath for the electrodeposition of metal comprising an aqueous solution providing ions of the metal to be deposited and metal starchate in which the metal is attached in the 2-position in the starch molecule, as an addition agent.

4. A plating bath for the electrodeposition of metal comprising an aqueous solution providing ions of the metal to be deposited and a colloidal solution of an alkali metal starchate in sufficient amount to inhibit the building up of large crystals of metal during the deposition.

5. A plating bath for the electrodeposition of metal comprising an aqueous solution providing ions of the metal to be deposited by electrolysis and including as an addition agent for producing bright, smooth metal coatings an aqueous colloidal solution of metal starchate in which the metal is attached in the 2-position in the starch molecule.

6. An electroplating bath comprising an aqueous solution providing ions of nickel to be deposited by electrolysis and a metal starchate compound in which the metal is that being deposited.

7. In a process for the electrodeposition of metal, the step comprising depositing said metal from an aqueous electrolyte solution of a salt thereof in the presence of an addition agent consisting of a metal starchate of the metal being deposited.

8. In a process for the electrodeposition of metal, the step comprising depositing said metal from an aqueous electrolyte solution of a salt thereof in the presence of an alkali metal starchate compound comprising the reaction product of starch and an alkali metal.

9. In a process of electrodeposition of metal, the step comprising depositing said metal from an aqueous electrolyte solution of a salt thereof in the presence of a colloidal aqueous suspension of a metal starchate compound in which the metal is attached in the 2-position in the starch molecule.

10. A process for the electrodeposition of metal

which comprises passing electric current from an anode to a cathode through an aqueous electrolyte bath in the presence of a metal starchate compound in which the metal is attached in the 2-position in the starch molecule incorporated in said electrolyte bath.

11. An electrolyte composition for use in electroplating metals, comprising an aqueous solution of an ionizable compound of the metal to be deposited and as an addition agent a metal starchate of said metal being plated out.

12. An electrolyte for use in the electrodeposition of metal, comprising an aqueous solution of an ionizable compound of the metal to be deposited and sufficient alkali metal starchate to produce a bright, adherent plate.

13. A plating bath comprising nickel sulfate, nickel chloride, boric acid, and sodium starchate dissolved in a sufficient quantity of water to provide a bath of the desired concentration.

14. A plating bath comprising by weight nickel sulfate 135 to 165 parts, nickel chloride 20 to 30 parts, boric acid 20 to 40 parts, and sodium starchate 5 to 25 parts.

15. A plating bath comprising nickel sulfate, nickel chloride, boric acid, nickel starchate, and water in quantity sufficient to provide a bath of the desired concentration.

16. A plating bath comprising by weight nickel sulfate 135 to 165 parts, nickel chloride 20 to 30 parts, boric acid 20 to 40 parts, and nickel starchate 5 to 25 parts.

17. A plating bath comprising sodium cyanide, cadmium hydroxide, sodium sulfate, sodium starchate, and water in quantity sufficient to provide a bath of the desired concentration.

18. A plating bath comprising by weight sodium cyanide 100 to 125 parts, cadmium hydroxide 35 to 50 parts, sodium sulfate 40 to 55 parts, and sodium starchate 10 to 25 parts, said sodium starchate content being based on the dry basis.

19. A plating bath comprising sodium cyanide, cadmium hydroxide, sodium sulfate, cadmium starchate, and water in quantity sufficient to provide a solution of the desired concentration.

20. A plating bath comprising by weight sodium cyanide 100 to 125 parts, cadmium hydroxide 35 to 50 parts, sodium sulfate 40 to 55 parts, and cadmium starchate 10 to 25 parts, said cadmium starchate content being based on the dry basis.

21. A plating bath comprising copper cyanide, sodium cyanide, sodium carbonate, sodium starchate, and water in quantity sufficient to provide a bath of the desired concentration.

22. A plating bath comprising by weight copper cyanide 100 to 120 parts, sodium cyanide 150 to 160 parts, sodium carbonate 25 to 30 parts, and sodium starchate 5 to 20 parts, said sodium starchate content being based on a 50% aqueous solution basis.

KENNETH M. GAVER.